

April 18, 1961

A. G. ROCCHINI ET AL

2,979,890

RESIDUAL FUELS

Filed Dec. 10, 1957



INVENTORS  
ALBERT G. ROCCHINI  
CHARLES E. TRAUTMAN  
BY

*Harold Blaustein*  
ATTORNEY

2,979,890

## RESIDUAL FUELS

Albert G. Rochini, Springdale, and Charles E. Trautman, Cheswick, Pa., assignors to Gulf Research & Development Company, Pittsburgh, Pa., a corporation of Delaware

Filed Dec. 10, 1957, Ser. No. 701,847

5 Claims. (Cl. 60—35.6)

This invention relates to vanadium-containing petroleum fuels. More particularly, it is concerned with rendering non-corrosive those residual fuels which contain such an amount of vanadium as normally to yield a corrosive vanadium-containing ash upon combustion.

It has been observed that when a residual type fuel oil containing substantial amounts of vanadium is burned in furnaces, boilers and gas turbines, the ash resulting from combustion of the fuel oil is highly corrosive to materials of construction at elevated temperatures and attacks such parts as boiler tubes, hangers, turbine blades, and the like. These effects are particularly noticeable in gas turbines. Large gas turbines show promise of becoming an important type of industrial prime mover. However, economic considerations based on the efficiency of the gas turbine dictate the use of a fuel for this purpose which is cheaper than a distillate diesel fuel; otherwise, other forms of power such as diesel engines become competitive with gas turbines.

One of the main problems arising in the use of residual fuel oils in gas turbines is the corrosiveness induced by those residual fuels containing sufficient amounts of vanadium to cause corrosion. Where no vanadium is present or the amount of vanadium is small, no appreciable corrosion is encountered. While many residual fuel oils as normally obtained in the refinery contain so little vanadium, or none, as to present no corrosion problems, such non-corrosive fuel oils are not always available at the point where the oil is to be used. In such instance, the cost of transportation of the non-corrosive oil to the point of use is often prohibitive, and the residual oil loses its competitive advantage. These factors appear to militate against the extensive use of residual fuel oils for gas turbines. Aside from corrosion, the formation of deposits upon the burning of a residual fuel in a gas turbine may result in unbalance of the turbine blades, clogging of openings and reduced thermal efficiency of the turbine.

Substantially identical problems are encountered when using a solid residual petroleum fuel containing substantial amounts of vanadium. These fuels are petroleum residues obtained by known methods of petroleum refining such as deep vacuum reduction of asphaltic crudes to obtain solid residues, visbreaking of liquid distillation bottoms followed by distillation to obtain solid residues, coking of liquid distillation bottoms, and the like. The solid residues thus obtained are known variously as petroleum pitches or cokes and find use as fuels. Since the vanadium content of the original crude oil tends to concentrate in the residual fractions, and since the processing of the residual fractions to solid residues results in further concentration of the vanadium in the solid residues, the vanadium corrosion problem tends to be intensified in using the solid residues as fuel.

The vanadium-containing ash present in the hot flue gas obtained from the burning of a residual fuel containing substantial amounts of vanadium compounds causes "catastrophic" corrosion of the turbine blades and other

metal parts in a gas turbine. The corrosive nature of the ash appears to be due to its vanadium oxide content. Certain inorganic compounds of vanadium, such as vanadium oxide ( $V_2O_5$ ), which are formed on combustion of a residual fuel oil containing vanadium compounds, vigorously attack various metals, their alloys, and other materials at the elevated temperatures encountered in the combustion gases, the rate of attack becoming progressively more severe as the temperature is increased. The vanadium-containing ash forms deposits on the parts affected and corrosively reacts with them. It is a hard, adherent material when cooled to ordinary temperatures.

It has now been discovered that residual petroleum fuels containing vanadium in an amount sufficient to yield

a corrosive vanadium-containing ash upon combustion can be rendered substantially less corrosive, notwithstanding the normally corrosive vanadium content, by incorporating therein to form a uniform blend a small amount, sufficient to retard the corrosiveness of the ash, of an alkali metal tungstate. In the fuel compositions of the invention, corrosion due to the vanadium-containing ash is substantially retarded.

In the accompanying drawing, the single figure shows an apparatus for testing the corrosivity of residual fuel oil compositions.

The type of residual fuel oils to which the invention is directed is exemplified by No. 5, No. 6 and Bunker "C" fuel oils which contain a sufficient amount of vanadium to form a corrosive ash upon combustion. These are

residual type fuel oils obtained from petroleum by methods known to the art. For example, residual fuel oils are obtained as liquid residua by the conventional distillation of total crudes, by atmospheric and vacuum reduction of total crudes, by the thermal cracking of topped

crudes, by visbreaking heavy petroleum residua, and other conventional treatments of heavy petroleum oils. Residua thus obtained are sometimes diluted with distillate fuel oil stocks, known as "cutter" stocks, and the invention also includes a residual fuel oils so obtained,

provided that such oils contain sufficient vanadium normally to exhibit the corrosion characteristics described herein. It should be understood that distillate fuel oils themselves contain either no vanadium or such small amounts as to present no problem of corrosion. The total ash from commercial residual fuel oils usually ranges from about 0.02 to 0.2 percent by weight. The vanadium pentoxide ( $V_2O_5$ ) content of such ashes ranges from zero to trace amounts up to about 5 percent by weight for low vanadium stocks, exhibiting no significant

vanadium corrosion problem, to as much as 85 percent by weight for some of the high vanadium stocks, exhibiting severe corrosion.

The type of vanadium-containing solid residual fuels to which the invention is directed is exemplified by the coke

obtained in known manner by the delayed thermal coking or fluidized coking of topped or reduced crude oils and by the pitches obtained in known manner by the deep vacuum reduction of asphaltic crudes to obtain solid residues. These materials have ash contents of the order

of 0.18 percent by weight, more or less, and contain corrosive amounts of vanadium when prepared from stocks containing substantial amounts of vanadium. A typical pitch exhibiting corrosive characteristics upon combustion had a softening point of 347° F. and a vanadium content, as vanadium, of 578 parts per million.

The corrosion retarding additive of the invention is, as has been stated, an alkali metal tungstate. The additive is employed in the dry form or as a water solution. The alkali metal tungstates include the sodium, potassium, lithium, rubidium and cesium tungstates in any of the ortho, meta or para tungstate forms. Because of

their availability and relatively low cost, the sodium and potassium tungstates are preferred.

When employing in residual fuels the dry alkali metal tungstates, it is desirable to use the finely-divided salts. However, the degree to which the salts are subdivided is not critical. One requirement for using a finely-divided material is based upon the desirability of forming a fairly stable dispersion or suspension of the salts when blended with a residual fuel oil. Furthermore, the more finely-divided materials are more efficient in forming uniform blends and rendering non-corrosive the relatively small amounts of vanadium in a residual fuel, whether the fuel be solid or liquid. The dry salts are therefore employed in a particle size range of less than 250 microns, preferably less than 50 microns. However, since the alkali metal tungstates are soluble in water, it is unnecessary to employ the finely divided dry additives when it is desired to employ water solutions thereof. Thus, the salts can be dissolved in water to form more or less concentrated solutions and the solutions then are emulsified in the fuel.

In the practice of the invention with vanadium-containing residual fuel oils, the additive is uniformly blended with the oil in proportion to the vanadium content thereof. This is accomplished by suspending the finely-divided dry salts in the oil, as has been indicated above, or by emulsifying or dispersing a water solution of the salts in the oil. If desired, suitable surface active agents, such as sorbitan monooleate and monolaurate and the ethylene oxide condensation products thereof, glycerol monooleate, and the like, which promote the suitability of the suspensions or emulsions can be employed.

In the practice of the invention with the solid residual fuels, incorporation of the additive of the invention is accomplished in several ways. The additive can be suspended or emulsified in the liquid vanadium-containing residual stocks or crude oil stocks from which the solid residual fuels of the invention are derived, and the mixture can then be subjected to the refining process which will produce the solid fuel. For example, in the production of a pitch by the deep vacuum reduction of an asphaltic crude oil, sodium ortho tungstate or a solution thereof in water is slurried with the oil in proportion to the vanadium content thereof, and the whole subjected to deep vacuum reduction to obtain a pitch containing the additive uniformly dispersed therein. As still another alternative, particularly with a pitch which is withdrawn in molten form from the processing vessel, the additive can be mixed with the molten pitch and the mixture allowed to solidify after which it is ground to the desired size.

In the case of either liquid or solid residual fuels, the additive can be separately fed into the burner as the dry salts, an oil dispersion thereof or a water solution thereof. In any such case, it is preferred to meter the additive into the fuel line just prior to the combustion zone. In a gas turbine plant where the heat resisting metallic parts are exposed to hot combustion gases at temperatures of the order of 1200° F. and above, the additive can be added separately from the fuel either prior to or during combustion itself, or even subsequent to combustion. However, it may specifically be added, whether in admixture with or separately from the fuel, the additive is introduced into said plant upstream of the heat resisting metal parts to be protected from corrosion.

The alkali metal tungstates are employed in a small amount with respect to the vanadium-containing residual fuel, sufficient to retard the corrosiveness of the ash. Although the exact amount of additive to use will vary in accordance with the vanadium content of the specific residual fuel employed, as will be understood by those skilled in the art, in general a reduction in corrosivity is already observed with an amount of the alkali metal tungstate sufficient to yield about 1 atom weight

of the tungsten present in the additive per atom weight of vanadium in the residual fuel. However, corrosivity is minimized when an amount of additive is employed yielding from about 3 to about 6 atom weights of tungsten per atom weight of vanadium in the residual fuel, and appears to be at a minimum at an atom weight ratio of tungsten to vanadium of 3:1.

The following specific examples are further illustrative of the invention.

- 10 A series of residual fuel oil compositions employing varying amounts of additive are made up and tested under conditions of burning residual fuel oils in a gas turbine. Identical tests are run on the residual fuel oil containing no additive. In the testing the apparatus shown in the drawing is employed. As shown therein, the residual oil under test is introduced through line 10 into a heating coil 11 disposed in a tank of water 12 maintained at such temperature that the incoming fuel is preheated to a temperature of approximately 212° F.
- 15 From the heating coil 11 the preheated oil is passed into an atomizing head designated generally as 13. The preheated oil passes through a passageway 14 into a nozzle 15 which consists of a #26 hypodermic needle of approximately 0.008 inch I.D. and 0.018 inch O.D. The tip of the nozzle is ground square and allowed to project slightly through an orifice 16 of approximately 0.020 inch diameter. The orifice is supplied with 65 p.s.i.g. air for atomization of the fuel into the combustion chamber 21. The air is introduced through line 17, preheat coil 18 in tank 12, and air passageways 19 and 20 in the atomizing head 13. The combustion chamber 21 is made up of two concentric cylinders 22 and 23, respectively, welded to two end plates 24 and 25. Cylinder 22 has a diameter of 2 inches and cylinder 23 has a diameter of 3 inches; the length of the cylinders between the end plates is 8½ inches. End plate 24 has a central opening 26 into which the atomizing head is inserted. End plate 25 has a one (1) inch opening 27 covered by a baffle plate 28 mounted in front of it to prevent direct blast of flame on the test specimen 29. Opening 27 in end plate 25 discharges into a smaller cylinder 30 having a diameter of 1½ inches and a length of 6 inches. The specimen 29 is mounted near the downstream end of the cylinder approximately 1¾ inches from the outlet thereof. Combustion air is introduced by means of air inlet 31 into the annulus between cylinders 22 and 23, thereby preheating the combustion air, and then through three pairs of ¾ inch tangential air inlets 32 in the inner cylinder 22. The first pair of air inlets is spaced ¼ inch from end plate 24; the second pair ¾ inch from the first; and the third 3 inches from the second. The additional heating required to bring the combustion products to test temperature is supplied by an electric heating coil 33 surrounding the outer cylinder 23. The entire combustion assembly is surrounded by suitable insulation 34.
- 20 The test specimen 29 is a metal disc one inch in diameter by 0.125 inch thick, with a hole in the center by means of which the specimen is attached to a tube 35 containing thermocouples. The specimen and tube assembly are mounted on a suitable stand 36.
- 25 In conducting a test in the above-described apparatus, a weighed metal specimen is exposed to the combustion products of a residual fuel oil, the specimen being maintained at a selected test temperature of, for example, 1350°, 1450° or 1550° F. by the heat of the combustion products. The test is usually run for a period of 100 hours with the rate of fuel feed being ½ pound per hour and the rate of atomizing air feed being 2 pounds per hour. The combustion air entering through air inlet 31 is fed at 25 pounds per hour. At the end of the test run the specimen is reweighed to determine the weight of deposits and is then descaled with a conventional alkaline descaling salt in molten condition at 4750° C. After descaling, the specimen is dipped in 6 N hydrochloric acid containing a conventional pickling inhibitor, and is
- 30
- 35
- 40
- 45
- 50
- 55
- 60
- 65
- 70
- 75

then washed, dried and weighed. The loss in weight of the specimen after descaling is the corrosion loss.

The compounded and uncompounded residual fuel oils are tested in the apparatus just described using a 25-20 stainless steel as the test specimen. The tests are run for 100 hours at a temperature of 1450° F. under the conditions described above. The residual oil employed as a base fuel has the following inspection:

|                         |      |
|-------------------------|------|
| Gravity, ° A.P.I.       | 20.6 |
| Viscosity, Furol, Sec.: |      |
| 77° F.                  | 74.3 |
| 122° F.                 | 25.4 |
| Flash, OC: ° F.         | 255  |
| Fire, OC: ° F.          | 295  |
| Sulfur, B: percent      | 1.6  |
| Ash: percent            | 0.04 |
| Vanadium: p.p.m. of oil | 182  |
| Sodium: p.p.m. of oil   | 2    |

The alkali metal tungstate employed in this series of runs is sodium para tungstate ( $Na_6W_7O_{24} \cdot 16H_2O$ ).

The following table shows the make-up and the reduction in corrosion and deposits obtained in the tests.

TABLE I

|                                                 | Fuel (Blank) | Ex. 1        | Ex. 2   | Ex. 3   | Ex. 4   |
|-------------------------------------------------|--------------|--------------|---------|---------|---------|
| Amount of Additive:                             |              |              |         |         |         |
| Percent by Wt. of Fuel                          | 0            | 0.15         | 0.2     | 0.3     | 0.7     |
| Atom Ratio, W:V                                 | 0            | 1.5:1        | 2:1     | 3:1     | 6:1     |
| Corrosion, Wt. Loss of Specimen, Mg./Sq. In.    | 1,580        | 128          | 97      | 7       | 28      |
| Reduction in Corrosion Due to Additive, Percent |              | 92           | 94      | 99.5    | 99      |
| Deposits on Specimen, Mg./Sq. In.               | 1,130        | 276          | 115     | 119     | 164     |
| Texture of Deposits                             | Hard Scale   | Hard Deposit | Powdery | Powdery | Powdery |

It is apparent from the foregoing data that sodium tungstate is an efficient corrosion inhibitor and is most effective when employed in an amount yielding an atom weight ratio, W:V, of 3:1. Similar results are obtained employing the other alkali metal tungstates disclosed herein.

The following example is illustrative of the use of the additive of the invention with solid residual fuels.

#### Example 5

Melt a solid petroleum pitch obtained from the deep vacuum reduction of an asphaltic crude. This pitch has a softening point of 347° F. and a vanadium content of 578 parts per million. While the pitch is in molten form, add and uniformly blend therein with stirring 1.25 percent by weight of finely powdered dry potassium ortho tungstate ( $K_2WO_4 \cdot 2H_2O$ ). Upon cooling and solidifica-

tion, grind the mixture to about 150 mesh. The resulting fuel has an atom weight ratio, W:V, of 3:1.

A typical analysis of the 25-20 stainless steel employed in the testing described is shown in the following table in percent by weight.

Table II

|       | 25-20   |
|-------|---------|
| Cr    | 25      |
| Ni    | 20      |
| 10 C  | 0.08    |
| Mn    | 2.0     |
| Si    | 1.5     |
| S     | 0.03    |
| P     | 0.04    |
| 15 Fe | Balance |

Resort may be had to such modifications and variations as fall within the spirit of the invention and the scope of the appended claims.

We claim:

20 1. A fuel composition comprising a uniform blend of a residual petroleum fuel yielding a corrosive vanadium-containing ash upon combustion and an amount of an alkali metal tungstate sufficient to yield from about 3 to about 6 atom weights of tungsten per atom weight of vanadium in said fuel.

2. The fuel composition of claim 1, wherein the fuel is a solid residual fuel.

3. A fuel composition comprising a uniform blend of a residual petroleum fuel oil yielding a corrosive vanadium-containing ash upon combustion and an amount of a sodium tungstate sufficient to yield from about 3 to about 6 atom weights of tungsten per atom weight of vanadium in said fuel oil.

4. The fuel composition of claim 3, wherein the tungstate is sodium paratungstate.

5. In a gas turbine plant in which a fuel oil containing vanadium is burned and which includes heat resistant metallic parts exposed to hot combustion gases and liable to 40 be corroded by the corrosive vanadium-containing ash resulting from the combustion of said oil, the method of reducing said corrosion which comprises introducing into said plant upstream of said parts an amount of an alkali metal tungstate sufficient to yield from about 3 to about 6 atom weights of tungsten per atom weight of vanadium in said fuel oil.

#### References Cited in the file of this patent

##### FOREIGN PATENTS

|    |           |               |                |
|----|-----------|---------------|----------------|
| 50 | 12,401    | Great Britain | Oct. 19, 1888  |
|    | 697,101   | Great Britain | Sept. 16, 1953 |
|    | 761,378   | Great Britain | Nov. 14, 1956  |
|    | 781,581   | Great Britain | Aug. 21, 1957  |
| 55 | 1,117,896 | France        | Mar. 5, 1956   |
|    | 498,777   | Belgium       | Nov. 14, 1950  |